

## UNITED STATES PATENT OFFICE

2,497,538

FLUXES FOR USE IN THE TREATMENT OF  
LIGHT METALS

Edward Frederick Emley and Alfred C. Jessup,  
Clifton Junction, near Manchester, England,  
assignors to Magnesium Elektron Limited, London, England, a British company

No Drawing. Application August 2, 1947, Serial  
No. 765,802. In Great Britain August 29, 1946

3 Claims. (Cl. 75—87)

1

This invention relates to fluxes for use in the treatment of light metals consisting of magnesium, magnesium base alloys, and aluminium base alloys containing magnesium all hereinafter included in the term "metal."

Many such fluxes have heretofore been proposed and those mainly used on a large commercial scale comprise two main kinds namely:

(a) An inspissated flux intended for refining the metal as well as for preventing oxidation and the main characteristics of which are described in British Patent No. 539,024; and

(b) A thinly fluid or non-inspissated flux of low melting point intended mainly for protecting the metal against oxidation during melting, and examples of this type and its main characteristics are described in British Patent No. 539,023.

The present invention is concerned with fluxes of type (a).

These fluxes all contain chlorides and as is well known proper care must be exercised both in selecting suitable compositions for the fluxes and also in their use in order to minimise contamination of the finished metal with chlorides which give rise to corrosion of the metal.

This difficulty is experienced with normal commercial magnesium alloys containing minor percentages of manganese, aluminium and zinc. We have also met with chloride contamination difficulties of a special nature when dealing with the magnesium base alloys described in British Patent No. 511,137 namely alloys containing a small percentage of zirconium in the absence of elements such as aluminium and silicon which form high melting point compounds with zirconium.

It has been the constant experience hitherto that magnesium alloys containing zirconium are difficult to prepare in a flux-free state, and work on this problem had resulted in the inventions forming the subject of co-pending British patent applications Nos. 7,227, 18,890 and 20,870, all of 1945, according to which it is proposed to effect alloying by means of zirconium fluoride dissolved in a molten bath of inert fluorides, or by potassium fluozirconates either with or without the presence of a chloride bath.

We have now found that even with the alloying methods described in these co-pending British applications it is very difficult to remove undesirable traces of chlorides which may be introduced by chlorides present in the alloying mixtures or which may be introduced after alloying

by the subsequent treatment with chloride-containing flux.

We have also found that a given quantity of included flux produces on exposure to damp air a much more conspicuous corrosion mark on magnesium-zinc-zirconium than on standard alloys. This is not due to a difference in corrosion resistance of the alloys, but is caused by local surface discolouration developing on the magnesium-zinc-zirconium alloys. In order therefore to reduce the incidence of these traces of flux below that in the standard alloys, as judged visually by the exposure in a humidity chamber of carefully machined sections of the alloys, we have had to devise methods of producing in magnesium-zinc-zirconium alloys a degree of freedom from traces of flux not previously realised in standard alloys.

We have also ascertained that when magnesium alloy scrap containing zirconium is remelted with normal fluxes a considerable amount of new contamination is invariably introduced. Although light in nature, this secondary contamination is widespread and renders the remelted alloy quite unfit for most commercial purposes.

It is also well known that the preparation of cerium-containing alloys in a flux-free state is a matter of considerable difficulty and inconvenience.

With a view to eliminating these residual traces of flux contamination in zirconium-containing and cerium-containing alloys, we have made extensive experiments on lines which have included the following:

1. Modification of known fluxes in various ways, for instance by use of fluxes in which the  $MgCl_2/CaF_2$  ratio is such as to produce a slight non-wetting action.
2. Modification of pouring technique, in particular by fitting special traps to the pouring lip of the crucible and special ingates to the mould.
3. Use of mechanical filters.
4. Use of special inhibitors to permit very careful cleaning of the metal surface before pouring and to form a strong coherent oxide tube during pouring.
5. Modification of the inert fluoride alloying bath.
6. Increase in settling time before pouring.
7. Settling under favourable temperature gradient in which the upper part of the metal is maintained at a higher temperature than the lower part during a settling period.

With the exception of (7) none of these methods has shown an appreciably beneficial effect.

In view of the slight improvement following

adoption of settling under a favourable temperature gradient, it was decided to investigate the possibility of preparing a special high density flux of the inspissated type for use with magnesium alloys containing zirconium. Whilst it is obvious that such fluxes must contain a high proportion of barium and/or strontium halides in order to attain the necessary high density, it is nevertheless essential that such fluxes should not only introduce no barium or strontium into the fluxed alloy, but should actually be able to remove barium and strontium already in the alloy at least partially during the fluxing process, since traces of barium and strontium are harmful to magnesium-zinc-zirconium alloys for certain purposes and particularly for preparation of sand castings.

It was also desirable that such fluxes should possess the following properties:

1. Suitability for use while stirring melts at fairly high temperatures (for example over 800° C.).
2. Suitability for use as an all purpose flux, i. e. for melting, refining, covering during superheating where required, and as a cover during pouring the metal.
3. Reduced hygroscopicity compared with standard fluxes (for example those of British Patent No. 539,024), since foundry conditions are frequently unsuitable for storing fluxes of a very hygroscopic nature.
4. Freedom from sodium salts so as to prevent the risk of introducing undesirable amounts of this element through interchange of radicals.
5. Inertness to rare earth metals where the fluxes are to be used for alloys containing rare earth metals.

We have found it possible to prepare the following four types of heavy fluxes, three of which possess special properties as indicated below in addition to the general properties of high density, power of removing strontium and barium, and the properties numbered (1), (2) and (3) above.

*Type 1.*—Standard heavy flux, i. e., suitable for puddling, refining and covering the alloys.

*Type 2.*—Flux with special suitability for remelting zirconium-containing alloy scrap (hereinafter termed superheavy flux).

*Type 3.*—Flux with special suitability for alloys containing rare earth metals with or without zirconium.

*Type 4.*—Non-hygroscopic flux.

The use of these fluxes in conjunction, where zirconium is to be introduced, with the alloying method disclosed in British patent application No. 7,227 of 1945, has enabled us to prepare alloys containing (a) zirconium, (b) zirconium and rare earth metals, and (c) rare earth metals, which are of an extremely high degree of freedom from flux.

We have found that in order to avoid the introduction by the flux of traces of barium or strontium into metal, where such traces are undesirable, or to remove or reduce the content of barium and strontium which may already be present in the metal, it is necessary for the flux either to contain no fluorides of barium or strontium or for magnesium chloride to be present in chemical excess of the fluorides of barium and strontium present. For example, two chemical equivalents of magnesium chloride for each equivalent of strontium or barium fluoride present will give good results.

We have ascertained that the inspissated fluxes of the present invention may be used in the treat-

ment of normal commercial type of magnesium base alloys, e. g. those containing magnesium and manganese, magnesium, aluminium and manganese, and magnesium, aluminium, zinc and manganese, and also with aluminium base alloys containing magnesium, with improved results, that is to say with an even greater degree of freedom from chlorides in the finished alloys than when using fluxes of the normal commercial types.

- 10 We have found that a protective base consisting of  $\text{BaCl}_2$ — $\text{MgCl}_2$ — $\text{KCl}$  in the approximate proportions of 50:38:12 is very satisfactory for preparation of the fluxes of the types 1 and 2. For maximum density we inspissate this with  $\text{BaF}_2$  which is added to the molten protective base, and the resulting product is cast into moulds, crushed, and milled. This "superheavy" flux has a density of 2.7 g. per cc. in comparison with standard fluxes of density 1.8 to 2.0 g. per cc. and consequently any inclusions of this flux which may be formed in the metal at any stage of the alloying process will have from five to ten times the settling rate of inclusions of standard flux of the same volume, when calculated according to Stokes' law. For this superheavy flux the whole or at least 75% of the inspissating agents consist of barium fluoride and/or strontium fluoride and the chlorides preferably comprise barium and/or strontium chloride in quantity at least equivalent to 40% barium chloride. Alternatively, where the highest density is not required, a standard type of flux may be produced by mixing the  $\text{BaF}_2$  with the milled protective base in powder form instead of by fusion, the density of the resulting flux being somewhat less (2.55 to 2.6 g. per cc.).
- 20 The permissible latitude in composition of this flux is, however, extremely narrow, the  $\text{BaF}_2$  content necessary to produce the required degree of inspissation being critical to 1 or 2% on either side of the optimum content, which we find may vary with the condition of the particular sample of protective base used and particularly with its degree of hydration.
- 30 With a view to increasing this latitude in composition and thereby rendering the production of a standard type of heavy flux practicable on a continuously operating plant, we have substituted  $\text{MgF}_2$  for  $\text{BaF}_2$  with considerable success. The density of this standard heavy flux (type 1) is 2.5 to 2.55 g. per cc. and therefore rather less than that of the "superheavy" flux, but we have found that this flux gives excellent results. To compensate for the slightly reduced density and to cheapen the product, we have also in certain cases introduced calcium chloride and sodium chloride into the protective base with satisfactory results, and we have also substituted (a)  $\text{CaF}_2$ , (b)  $\text{CaF}_2$  and  $\text{MgO}$  and (c)  $\text{MgO}$  for some, or even all, of the  $\text{MgF}_2$ , though in the latter case we prefer to prefuse the  $\text{MgO}$  into the protective base.
- 40 We have prepared satisfactory fluxes for use with zirconium alloys containing rare earth metals by inspissating the following protective base with  $\text{MgO}$  and/or  $\text{CaF}_2$ :

65  $50 \text{ BaCl}_2$   
 $25 \text{ CaCl}_2$   
 $15 \text{ NaCl}$   
 $10 \text{ KCl}$

- 70 but such fluxes possess inconveniently narrow permissible latitude in composition and we prefer, therefore, to inspissate this base with  $\text{MgF}_2$  which we have found provides a much wider latitude.
- 75 We have also succeeded in preparing a non-

hygroscopic flux from a protective base of  $\text{BaCl}_2$ ,  $\text{KCl}$  and  $\text{NaCl}$ . It was found that if  $\text{CaF}_2$ ,  $\text{BaF}_2$  or  $\text{SrF}_2$  were used as inspissating agents for the protective base, the resulting fluxes were all strongly non-wetting. If at least 75 per cent of the inspissating agents in the flux consist of  $\text{MgF}_2$ , the non-wetting was eliminated. Barium fluoride and strontium fluoride are preferably absent or at any rate constitute not more than 10% of the total inspissating agents. Preferably the whole of the inspissating effect for this purpose should be provided by  $\text{MgF}_2$  but if some proportion of other inspissating agent is present this should preferably not comprise any other fluoride. The resulting flux was very satisfactory in behaviour except in its lack of ability rapidly to extinguish burning metal which rendered the flux unsuitable for use in melting magnesium alloys. By prefusion of the constituents of the protective base it was found possible to overcome this disadvantage and so produce a completely non-hygroscopic flux which was entirely satisfactory as a flux in all respects.

We have found that the  $\text{BaCl}_2$  may, if desired be replaced at least partially by  $\text{SrCl}_2$  in any of the heavy fluxes described.

The fluxes may contain minor proportions of "inert impurities" such as  $\text{SiO}_2$ ,  $\text{Fe}_2\text{O}_3$ ,  $\text{Al}_2\text{O}_3$ ,  $\text{CaO}$  and carbon, which may be present either as impurities in the constituents of the flux or may be added for their inspissating action in amounts up to 35%.

Certain variations may be used both in the ingredients of the inspissated fluxes according to the present invention, and also in their relative proportions, but the following features must be taken into consideration.

1. The strontium chloride and/or barium chloride may be wholly replaced by strontium fluoride and/or barium fluoride. In this case the inspissated flux must contain at least 12% of barium fluoride, i. e. equivalent to 20% of barium chloride based on the total flux which is approximately equivalent to 25% of barium chlorides based on the weight of the chlorides alone. Alternatively the flux may contain both barium and strontium fluorides in amounts equivalent to at least 12% barium fluoride, reckoning 1% strontium fluoride equivalent to 0.35% barium fluoride.

2. If desired the strontium and/or barium chloride may be partly replaced by strontium and/or barium fluoride. In this case the barium and strontium halides must be equivalent in total to at least 20% (of the total flux) of barium chloride reckoning 1% barium chloride equivalent to 1.4% strontium chloride, 0.6% barium fluoride, and 1.6% strontium fluoride.

3. In the flux incorporates strontium and/or barium fluoride it must also include at least a stoichiometrically chemical equivalent of magnesium chloride to avoid the reduced wetting tendency and to prevent entry of strontium and barium into the metal in cases where this is not desirable.

4. The chlorides in the flux when melted alone, apart from the inspissating agents, should have a liquidus temperature not greater than  $750^\circ\text{C}$ ., and preferably not greater than  $610^\circ\text{C}$ ., that is to say a slightly greater liquidus temperature can be tolerated when the chlorides are used in an inspissated flux for refining and covering than when used alone as a melting flux.

5. The inspissated flux will consist solely of chlorides and fluorides of alkali metals and al-

kaline earth metals including magnesium together with, if desired, substantially inert oxides suitable for use as inspissating agents.

6. The quantity of inspissating agents, that is to say the fluoride and/or oxides, must be sufficient to cause the flux to produce a pasty viscous cover on the surface of the molten metal at  $750^\circ\text{C}$ .

7. If calcium chloride and magnesium chloride are absent, then at least 75% of the inspissating agents should consist of magnesium fluoride; other fluorides should preferably be absent and the protective base of the flux should preferably be prefused.

8. Preferably, if strontium and/or barium chloride are absent, the strontium and/or barium fluoride is/are prefused with one or more of the chlorides.

9. Preferably sodium and potassium fluorides are omitted from the flux, but these fluorides can be tolerated to some extent if sufficient magnesium chloride is present to avoid contamination of the metal by sodium and potassium and to prevent the reduced wetting effect.

10. The density of the fluxes of the present invention is at least 2.2 and preferably at least 2.4.

According to the present invention therefore the fluxes are composed as described under (a) below or in the modified form described under (b) produced by wholly or partly replacing the barium chloride and/or strontium chloride by barium fluoride and/or strontium fluoride.

(a) The flux contains at least two chlorides of the group consisting of the chlorides of the alkali and alkaline earth metals including magnesium, at least 25% of the chlorides being barium chloride, together with a sufficient proportion of one or more inspissating agents (other than barium fluoride and strontium fluoride) to enable the flux to provide a pasty viscous covering on the surface of the molten metal at  $750^\circ\text{C}$ ., the flux having a specific gravity of at least 2.2 at  $800^\circ\text{C}$ .; the barium chloride being partly or wholly replaceable by strontium chloride reckoning 1% strontium chloride equivalent to 0.7% barium chloride.

(b) The modified flux contains one or more of the salts of the group consisting of barium chloride, barium fluoride, strontium chloride, and strontium fluoride, including at least one of these fluorides, the total quantity of these salts being equivalent to at least 20% barium chloride reckoning 1% barium chloride equivalent to 1.4% strontium chloride, 0.6% barium fluoride, or 1.6% strontium fluoride, the flux also containing magnesium chloride in quantity at least stoichiometrically equivalent to the barium fluoride and/or strontium fluoride and having a specific gravity of at least 2.2 at  $800^\circ\text{C}$ . and being adapted to produce a pasty viscous cover on the metal at  $750^\circ\text{C}$ .

In addition to the  $\text{SrCl}_2$  and/or  $\text{BaCl}_2$  present in all fluxes, the following groups of additional chlorides and inspissating agents give fluxes which are particularly suitable for the purposes cited.

Type 2.—(For alloys containing zirconium): Chlorides of Mg and K with or without minor proportions of chlorides of Ca and Na, together with one or more fluorides selected from the group  $\text{MgF}_2$ ,  $\text{CaF}_2$  and  $\text{BaF}_2$  with or without minor amounts of  $\text{MgO}$ .

Type 3.—(For alloys containing rare earth elements with or without zirconium):

75 Chlorides of Ca, K and Na with one or more

fluorides selected from the group  $MgF_2$  and  $CaF_2$  with or without minor quantities of  $MgO$ .

Type 4.—(Non-hygroscopic flux):  
Chlorides of K and Na with  $MgF_2$ .

The density of the fluxes referred to above is the density at 800° C. and is measured by filling a container of known volume with molten flux at 800° C. and weighing.

The following ranges of compositions are particularly suitable for the special purposes indicated, the figures all indicating percentages by weight.

For alloys containing zirconium:

|                        | Best all-purpose flux and particularly for "Puddling" and removing Ba and Na | Best cover flux | "Super-heavy" (Scrap melting) | Cheaper fluxes suitable for same purposes as (A) and (B) and for Standard Alloys |       |       |
|------------------------|------------------------------------------------------------------------------|-----------------|-------------------------------|----------------------------------------------------------------------------------|-------|-------|
| Example reference..... | (A)                                                                          | (B)             | (C)                           | (D)                                                                              | (E)   | (F)   |
| $BaCl_2$ .....         | 20-45                                                                        | 20-45           | 20-45                         | 20-45                                                                            | 20-45 | 20-45 |
| $CaCl_2$ .....         |                                                                              |                 |                               | 5-20                                                                             | 5-20  |       |
| $MgCl_2$ .....         | 15-38                                                                        | 20-45           | 15-41                         | 0-10                                                                             | 0-10  | 15-42 |
| $KCl$ .....            | 4-17                                                                         | 4-16            | 4-17                          | 10-20                                                                            | 13-23 | 4-16  |
| $NaCl$ .....           |                                                                              |                 |                               | 14-26                                                                            | 17-30 |       |
| $BaF_2$ .....          |                                                                              | 18-22           | 21-27P                        |                                                                                  | 12-16 |       |
| $CaF_2$ .....          |                                                                              |                 |                               |                                                                                  |       | 18-38 |
| $MgF_2$ .....          | 18-30                                                                        |                 |                               | 16-30                                                                            |       |       |
| $MgO+CaO$ .....        |                                                                              |                 |                               | 5-17P                                                                            | 5-17P |       |
| Inert Impurities.....  |                                                                              |                 |                               |                                                                                  |       |       |

For various purposes:

|                        | Suitable for Standard Alloys | Suitable for Alloys containing rare earth metals with or without Zr | Non-dilute flux suitable for all alloys |       |       |
|------------------------|------------------------------|---------------------------------------------------------------------|-----------------------------------------|-------|-------|
| Example reference..... | (G)                          | (H)                                                                 | (I)                                     | (J)   | (K)   |
| $BaCl_2$ .....         | 15-35                        | 17-40                                                               | 20-45                                   | 15-35 | 30-50 |
| $CaCl_2$ .....         | 5-15                         | 4-10                                                                | 15-28                                   | 10-19 |       |
| $MgCl_2$ .....         | 15-24                        | 15-30                                                               |                                         |       |       |
| $KCl$ .....            | 3-7                          | 0-5                                                                 | 5-12                                    | 3-10  | 20-32 |
| $NaCl$ .....           | 4-12                         | 0-5                                                                 | 10-20                                   | 5-15  | 13-22 |
| $BaF_2$ .....          |                              | 15-25                                                               |                                         | 15-30 |       |
| $CaF_2$ .....          |                              |                                                                     |                                         |       | 13-21 |
| $MgF_2$ .....          | 18-20                        |                                                                     | 14-26                                   |       |       |
| $MgO+CaO$ .....        | 8-20                         | 8-16                                                                |                                         | 0-15  |       |
| Inert Impurities.....  | 15-35P                       |                                                                     |                                         |       |       |

The following specific compositions are quoted by way of further example, the small letter references corresponding with the similar above quoted capital letter references:

|                | (a) | (b) | (c) | (f) | (i) | (k) |
|----------------|-----|-----|-----|-----|-----|-----|
| $BaCl_2$ ..... | 38  | 39  | 38  | 35  | 38  | 40  |
| $CaCl_2$ ..... |     |     |     | 26  | 26  |     |
| $MgCl_2$ ..... | 28  | 30  | 29  | 26  |     | 26  |
| $KCl$ .....    | 9   | 10  | 9   | 9   | 10  | 26  |
| $NaCl$ .....   |     |     |     |     | 16  | 17  |
| $BaF_2$ .....  |     | 21  | 24P |     |     |     |
| $CaF_2$ .....  |     |     |     | 30  |     |     |
| $MgF_2$ .....  | 25  |     |     |     | 20  | 17  |
| $MgO$ .....    |     |     |     |     |     |     |

In all the above quoted examples the letter "P" means that the substance concerned is pre-fused with the chloride mixture.

We claim:

1. An inspissated flux for use in the treatment of magnesium and magnesium base alloys consisting of at least one halide selected from the group consisting of the chlorides and fluorides of barium and strontium, in total amount at least equivalent to 20% barium chloride reckoning 1% barium chloride equivalent to 1.4% strontium chloride, 0.6% barium fluoride, or 1.6% strontium fluoride, at least one chloride selected from the group consisting of the chlorides of calcium, mag-

nesium, and the alkali metals, said flux containing at least two of the aforementioned chlorides, said flux including at least one inspissating agent selected from the group consisting of such oxides and fluorides including the said barium fluoride and strontium fluoride as are chemically inert to molten magnesium, the quantity of inspissating agents being between 13% and 43%, and such as to enable the flux to provide a pasty viscous cover on the surface of the molten metal at 750° C., the flux having a specific gravity of at least 2.2 at 800° C. and being substantially free from sodium fluoride.

2. An inspissated flux as claimed in claim 1 which includes at least one of the fluorides selected from the group consisting of barium fluoride and strontium fluoride, and magnesium chloride in quantity at least stoichiometrically equivalent to the barium and strontium fluorides.

3. An inspissated flux for use in the treatment of magnesium and magnesium base alloys consisting of barium chloride from 20% to 45%, magnesium chloride from 15% to 42%, potassium chloride from 4% to 16%, and the balance consisting of from 18% to 38% of at least one inspissating agent selected from the group consisting of calcium fluoride, magnesium fluoride and magnesium oxide, the flux having a specific gravity of at least 2.2 at 800° C.

EDWARD FREDERICK EMLEY.  
ALFRED C. JESSUP.

#### REFERENCES CITED

The following references are of record in the file of this patent:

#### UNITED STATES PATENTS

| Number    | Name          | Date          |
|-----------|---------------|---------------|
| 1,359,851 | Whitmyre      | Nov. 23, 1920 |
| 1,968,984 | Binder        | Aug. 7, 1934  |
| 1,980,152 | Beck          | Nov. 6, 1934  |
| 2,148,664 | Wille et al.  | Feb. 28, 1939 |
| 2,170,863 | Junker et al. | Aug. 29, 1939 |
| 2,261,906 | Nelson et al. | Nov. 4, 1941  |
| 2,286,869 | McDonald      | June 16, 1942 |
| 2,453,444 | Loonam        | Nov. 9, 1948  |

#### FOREIGN PATENTS

| Number  | Country       | Date          |
|---------|---------------|---------------|
| 489,700 | Great Britain | Aug. 2, 1938  |
| 503,953 | Great Britain | Apr. 12, 1939 |

#### OTHER REFERENCES

Ser. No. 387,769, "Light Metals and Their Alloys," Henry Lepp (A. P. C.), published May 4, 1943.